

## UNITED STATES PATENT OFFICE

RAYMOND J. NORTON, OF WASHINGTON, DISTRICT OF COLUMBIA, ASSIGNOR TO AMERICAN MAGNESIUM METALS CORPORATION, OF PITTSBURGH, PENNSYLVANIA, A CORPORATION OF DELAWARE

## LIGHT METAL ALLOY

No Drawing. Application filed November 28, 1930, Serial No. 498,912. Renewed April 23, 1932.

This invention relates to improvements in light metal alloys and particularly to an improved magnesium beryllium alloy.

The advantage of beryllium as an alloying component with other metals has heretofore been appreciated. It has been proposed, for example, to incorporate small amounts of beryllium with aluminum to form a binary and with aluminum and copper to form a ternary alloy. It has furthermore been found that by a special heat treatment the aluminum beryllium alloys may be considerably improved as to hardness and breaking strength.

It has also been proposed to produce magnesium beryllium alloys. This type of alloy would present decided advantages in view of its great lightness.

The method of producing magnesium beryllium alloys heretofore proposed consists essentially of reducing a double fluoride of beryllium to the molten condition and adding to this a certain quantity of molten magnesium. The theory of the process is that a certain quantity of the magnesium reduces beryllium fluoride with the formation of beryllium and magnesium fluoride. The quantity of magnesium added, therefore, is equal to that to be contained in the final alloy and that required to reduce the beryllium halide. Prior art disclosures on this indicate that the operation was carried out in an iron vessel and that the end product presented a decided tendency to stick to the iron.

The present method represents a simplified process of preparing a magnesium beryllium alloy by combining the pure metals out of contact with iron, or other alloying substances, and substantially out of contact with air. The invention will be more fully understood from a consideration of the specific method of making up the desired material.

An alloy of magnesium and beryllium has been made up by treating a predetermined quantity of pure magnesium with the desired amount of beryllium. In tests actually run 45 2.4 grams of magnesium were used with approximately .3 of a gram of beryllium. The analysis of the beryllium indicated that the metal was in a high state of purity. The analysis of the magnesium indicated very

slight traces of aluminum and iron. In making up the alloy a strong iron bomb was lined with a refractory of magnesium oxide which was baked at a high temperature for approximately two hours. In the bomb was placed the quantities of magnesium and beryllium stated above, after which the bomb was hermetically sealed.

The material in the bomb was then heated for a coming up period for about two hours at 950° C. It was then held at between 950° and 1000° C. for five hours.

It will be noted that inasmuch as the bomb was hermetically sealed and inasmuch as the magnesium forms a stable oxide in a nitride, the heat treatment may be considered to be carried out under non-oxidizing conditions. It is also to be noted that the heat treatment is carried out below the melting point of beryllium, which is generally considered to be about 1280° C. After the described treatments, that is to say after heating in excess of 900° for prolonged period of time, a single billet of metal was removed from the bomb. This material looked considerably like magnesium but was quite definitely harder and more resistant to corrosion than pure magnesium.

In order to establish the homogeneity of the material, small pieces were cut off each end of the billet and each of these pieces were dissolved in an equal quantity of hydrochloric acid. After dissolution of the two ends the solution was treated with ammonium chloride and ammonia and allowed to stand for a period of two hours, during which time beryllium hydroxide was precipitated. It was found that the quantities of beryllium in each of the pieces were substantially the same, indicating the homogeneous dispersion and/or diffusion of the beryllium in the magnesium.

It appears that the present method may be similar in mechanics of operation to the diffusion of one metal in another, as is found for example in calorizing and chromizing treatments. In any event, it has been found that a new metallic compound of magnesium and beryllium may be made up which presents physical characteristics differing and

distinguishing from the two metal components, and that this compound may be obtained without the necessity of reducing the beryllium to the molten condition. In view of the conditions of the treatment it is also apparent that the characteristics of the final metallic substance are not dependent upon the formation of an iron beryllium alloy for, due to the fact that the operation is carried out out of contact with iron, the incorporation of this metal in the final alloy is precluded.

It will be appreciated therefore that the present process provides a method of readily and simply obtaining an improved alloy or metallic compound of magnesium and beryllium. The process involves only a simple heat treatment at relatively low temperatures and insures the formation of a final product which is characterized by desirable physical properties. Therefore, while a specific process has been described, it is to be understood that this is given merely as an example of one method of incorporating the principles disclosed herein and the invention is not to be considered restricted to the particular method of treatment except as such restrictions are clearly imposed by the appended claims.

30. I claim:

1. The method of making an alloy of magnesium and beryllium which comprises heating substantially pure magnesium and beryllium out of contact with air and above the melting point of magnesium for a prolonged period of time.

2. The method of making an alloy of magnesium and beryllium comprising heating the substantially pure metals out of contact with air for a prolonged period at a temperature above the melting point of magnesium but below the melting point of beryllium.

3. The method of making an alloy of magnesium and beryllium which comprises heating substantially pure magnesium and beryllium, above the melting point of magnesium for a prolonged period of time, out of contact with air in a vessel, the portion of which is in contact with the magnesium and beryllium being formed of material other than iron.

In testimony whereof I affix my signature.  
RAYMOND J. NORTON.